# EUROPEAN PATENT SPECIFICATION

(11) **EP 3 080 339 B1**
(45) Date of publication and mention of the grant of the patent: **13.05.2020**
(21) Application number: 14868852.6
(22) Date of filing: 11.12.2014
(51) Int. Cl.: C25D 5/44, C25D 3/22, C25D 3/44, C25D 3/56, C25D 5/10, F01D 5/28, C23C 18/54, C25D 3/66

(54) **HIGH PURITY ALUMINUM COATING WITH ZINC SACRIFICIAL UNDERLAYER FOR ALUMINUM ALLOY FAN BLADE PROTECTION**
HOCHREINE ALUMINIUMBESCHICHTUNG MIT ZINKOPFERUNTERSCHICHT ZUM SCHUTZ VON ALUMINIUMLEGIERUNGSGEBLÄSESCHAUFEL
REVÊTEMENT D'ALUMINIUM À HAUTE PURETÉ COMPRENANT UNE SOUS-COUCHE SACRIFICIELLE DE ZINC POUR LA PROTECTION D'UNE PALE DE VENTILATEUR EN ALLIAGE D'ALUMINIUM

(30) Priority: 11.12.2013 US 201361914543 P
(43) Date of publication of application: 19.10.2016
(73) Proprietor: United Technologies Corporation, Farmington, CT 06032 (US)
(72) Inventor: CHEN, Lei, South Windsor, Connecticut 06074 (US)
(74) Representative: Dehns
(86) International application number: PCT/US2014/069651
(87) International publication number: WO 2015/089245

(56) References cited:
- WO-A1-2014/099348
- WO-A1-2014/150508
- DE-A1- 2 166 843
- US-A- 4 346 128
- US-A- 4 454 823
- US-A- 4 980 195
- US-A1- 2004 173 467
- US-A1- 2010 247 321
- US-A1- 2011 177 358
- US-A1- 2013 192 982

## Description

### BACKGROUND

The present disclosure relates to a coating system for providing protection to aluminum alloy components such as fan blades.

Aluminum alloys are extensively used in the aeronautical industry due to their high strength and low density. They are used to form turbine engine components such as fan blades. Pitting and intergranular corrosion of the aluminum alloys is one key risk to be mitigated to ensure reliability. It has been found that intermetallic particles are primarily responsible for susceptibility of the aluminum alloys to localized corrosion.

Additionally, use of aluminum alloys as the body of engine fan blades often requires a titanium leading edge to avoid erosion damage of the blade. However, factory isolated titanium leading edges may short in the field via tip rubs and may give rise to conductive contaminates (soot) and dielectric bond breakdown due to mechanical or electrical stresses, which may lead to an aggressive corrosion attack and even galvanic corrosion enabled by the coupling of very active aluminum alloy and more inert titanium alloys.

Aluminum alloy clad aluminum alloys provide higher resistance to pitting, in particular when the surface is protected with either a chromate conversion coating and/or a chromate primer. Further protection results from the sacrificial clad when the base alloy is exposed. Nonetheless, the mechanical cladding cannot be readily applied to parts with complex geometry such as engine fan blades.

Pure aluminum coating has been shown to be capable of protecting aluminum alloys and it can enable trivalent chromium processing as a green alternative to chromate conversion coatings. However, pure aluminum is not sacrificial to the alloy fan blade body. Document DE2166846 discloses aluminium coating for applications in the aeronautic, astronautic and automobile industries.

There remains a need for a way to protect aluminum alloys from pitting and intergranular corrosion using a barrier layer when the protection layer is intact while still retaining protection even when the barrier layer is broken to expose the base alloy.

### SUMMARY

In accordance with the present disclosure, there is provided a coating system for an aluminum component which broadly comprises a substrate formed from an aluminum material, a zinc material sacrificial layer deposited on the substrate, and an aluminum coating deposited over the zinc sacrificial layer. The substrate is a fan blade used in a turbine engine and the sacrificial layer has a thickness of less than 10 µm (10 microns) and said aluminum coating has a thickness in the range of from 5 µm to 50 µm (5 microns to 50 microns).

In another and alternative embodiment, the sacrificial layer may be formed from zinc.

In another and alternative embodiment, the sacrificial layer may be formed from a zinc alloy.

In another and alternative embodiment, the substrate may be formed from an aluminum alloy.

In another and alternative embodiment, the aluminum coating may be aluminum.

In another and alternative embodiment, the aluminum coating may be an electroplated aluminum coating.

Further, in accordance with the present disclosure, there is provided a method for forming a coating system which enhances resistance against corrosion which broadly comprises the steps of: providing a substrate formed from an aluminum material; forming a zinc material underlayer on a surface of the substrate; and forming an aluminum coating on the zinc material underlayer. The substrate is a fan blade used in a turbine engine and the sacrificial layer has a thickness of from about 0.01 µm (0.01 microns) to less than 10 µm (10 microns) and said aluminum coating has a thickness in the range of from 5 µm to 50 µm (5 microns to 50 microns).

In another and alternative embodiment, the underlayer forming step may comprise depositing a zinc or zinc alloy on the surface using at least one zincating process.

In another and alternative embodiment, the method may further comprise plating zinc or a zinc alloy onto the deposited zinc or zinc alloy.

In another and alternative embodiment, the aluminum coating forming step may comprise depositing aluminum or an aluminum alloy onto said underlayer.

In another and alternative embodiment, the aluminum coating forming step may comprise electroplating aluminum onto the underlayer.

In another and alternative embodiment, the coating forming step may comprise chromate conversion coating or trivalent chromium process (TCP) treatment of the aluminum coating as a passivation method.

Other details of the high purity aluminum coating with zinc sacrificial underlayer for aluminum alloy fan blade protection are set forth in the following detailed description and the accompanying drawings, wherein like reference numerals depict like elements.

### BRIEF DESCRIPTION OF THE DRAWINGS

FIG. 1 is a schematic representation of a coating system in accordance with the present disclosure;

FIG. 2 is a schematic representation of the protection rendered by the composite layers when the top coating fails; and

FIG. 3 is a TEM image of a composite Al-Zn sacrificial coating coated aluminum alloy.

### DETAILED DESCRIPTION

The present disclosure relates to applying a corrosion resistant aluminum coating with a sacrificial underlayer to protect aluminum alloy components, which are fan blades, from localized corrosion and galvanic corrosion. The sacrificial underlay, in addition to providing improved protection, enhances the adhesion of the aluminum coating. In order to gain full coverage of the aluminum alloy component, the aluminum coating may be applied by electrodeposition or by cathodic arc deposition.

Referring now to FIG. 1, there is shown a coating system 10 in accordance with the present invention. The coating system 10 includes a substrate 12 which may be formed from an aluminum alloy. For example, the substrate 12 may be formed from aluminum alloy 6061. The substrate 12 is a turbine engine fan blade.

Deposited onto the surface 14 of the substrate 12 is a sacrificial underlayer 16. The sacrificial underlayer 16 may be formed from pure zinc or a zinc alloy. The underlayer 16 may be deposited onto the surface using a zincating process, preferably multiple zincate processing. A zinc coating can be formed on aluminum alloys by an immersion coating process in which aluminum is chemically exchanged in solution. In the zincate process, the native oxide layer of aluminum is removed in an alkaline solution. The aluminum exposed thereby reacts with zincate ions in a zincate solution to form a zinc layer on the aluminum alloy substrate. This process is known in the industry. Other zincating processes can also be used. The sacrificial underlayer 16 formed from pure zinc or a zinc alloy displaces the native aluminum oxide that tends to weaken the bonding of a coating applied to the aluminum alloy forming the substrate 12.

Once a seed layer is deposited using the zincating process, a zinc or zinc alloy may be subsequently deposited to attain better control of the underlayer composition and mechanical strength, such as by electroplating, following optional anodic etching in the same solution used for the deposition. The zinc plating solution may be an ionic liquid or deep eutectic solvent solution, which is a non-acidic and basic solution to avoid attacking the base aluminum alloy. The solution can comprise choline chloride, zinc chloride, auxiliary solvents and additives. The molar ratio of the choline chloride and zinc chloride ranges from 0.5 to 3.5. Polar aprotic and polar protic solvents can be used to adjust the viscosity and conductivity of the plating bath. The solvents include formic acid, citric acid, isopropanol (IPA), water, acetic acid, glycine (aminoacetic acide) and ethylene glycol. Preferred auxiliary solvent content is from 10 to 80 vol% relative to the mixture of choline chloride and metal chlorides on a premixing basis. Examples of additives used to further improve the zinc underlayer properties include sodium dodecyl sulfate, fluorosurfactants, cetyl trimethylammonium bromide (CTAB), or cetyl, trimethylammonium chloride (CTAC).

The zinc plating solution allows for better control of the electrochemical etching of the zinc displacement layer 16 by eliminating spontaneous reaction occurring in traditional zinc plating solutions, containing either acidic or basic chemistry.

After the underlayer 16 has been formed on the substrate 12, an aluminum coating 18 is deposited onto the displacement layer 16. The aluminum coating 18 may be pure aluminum. Alternatively, for certain applications, the aluminum coating 18 may be an aluminum alloy which contains more than 50 wt% aluminum. The aluminum coating 18 may be electroplated aluminum formed using either triethyaluminium/toluene solutions, such as an electroplating solution available from ALUMIPLATE®, or in room temperature ionic liquids including Lewis acidic 1-ethyl-3-methylimidazolium chloride or 1-butyl-3-methylimidazolium chloride and an aluminum salt, for example. Forming an electroplated aluminum coating 18 produces a high purity, dense aluminum coating 18 with non-line-of-sight advantage compared with alternative technologies such as ion vapor deposition.

Referring now to FIG. 2, there is shown the protection rendered by the zinc or zinc alloy underlayer 16 when the top aluminum coating 18 fails such as by cracking. The top coating failure allows electrolytes to penetrate through the barrier layer, which would create a corrosive environment that could lead to corrosion damage of the base aluminum alloy. With the presence of a more active zinc underlayer, corrosion occurs on the sacrificial zinc layer to delay the attack of the base alloy to allow mitigation actions to be taken during next inspection and maintenance. It is also expected that the corrosion of the zinc layer would progress laterally as opposed to a much more aggressive damage penetrating the base alloy without the protection of the sacrificial layer.

Referring now to FIG. 3, there is shown a transmission electron microscopy (TEM) image of an aluminum alloy 6061 substrate having an aluminum coating plated from an ionic liquid. It is clear from this image that a thick zinc underlayer 16 is well adherent to the substrate 12. The zinc is extremely thin in this case, but can be made thicker with complete dense structure to meet durability design requirement, via zinc electroplating on this seed layer.

The zinc or zinc alloy underlayer 16 has a thickness of from about 0.01 µm (0.01 microns) to less than 10 µm (10 microns). The aluminum coating 18 has a thickness in the range of from 5 to 50 µm (5 to 50 microns).

The coating system 10 of the present disclosure provides a double protection for corrosion enabled by a top aluminum coating and a sacrificial underlayer on the aluminum alloy substrate. The coating system 10 also provides full coverage of an entire fan blade as a result of using non-line of sight coating application techniques. Still further, a dense and pure aluminum coating imparts more effective corrosion protection enabled by chromate treatment or trivalent chromium treatment containing inhibitors compared with aluminum alloys. Still further, a pure aluminum coating (1) is amenable to more benign conversion coating treatment, i.e. TCP, and (2) can reduce or eliminate fatigue debit resulting from an anodizing or pickling process applied to aluminum alloy conventionally. Still further, the displacement layer formed from zinc or a zinc alloy yields an adherent aluminum coating. Finally, the coating system 10 provides an enhanced resistance to pitting and intergranular corrosion.

There has been provided a high purity aluminum coating with a zinc sacrificial underlayer for aluminum alloy fan blade protection. While the high purity aluminum coating with zinc sacrificial underlayer for aluminum alloy fan blade protection has been described in the context of specific embodiments thereof, other unforeseen alternatives, modifications, and variations may become apparent to those skilled in the art having read the foregoing description. Accordingly, it is intended to embrace those alternatives, modifications, and variations as fall within the broad scope of the appended claims.

## Claims

1. A coating system for an aluminum component which comprises:
a substrate formed from an aluminum material;
a zinc material sacrificial layer deposited on said substrate; and
an aluminum coating deposited over said zinc sacrificial layer,
wherein said substrate is a fan blade used in a turbine engine, and
wherein said sacrificial layer has a thickness of less than 10 µm and said aluminum coating has a thickness in the range of from 5 µm to 50 µm.

2. The coating system of claim 1, wherein said sacrificial layer is zinc.

3. The coating system of claim 1, wherein said sacrificial layer is a zinc alloy.

4. The coating system of any preceding claim, wherein said substrate is an aluminum alloy.

5. The coating system of any preceding claim, wherein said aluminum coating is pure aluminum.

6. The coating system of any preceding claim, wherein said aluminum coating is an electroplated aluminum coating.

7. The coating system of any preceding claim, wherein said substrate is a turbine engine component.

8. A method for forming a coating system which enhances resistance against corrosion comprising the steps of:
providing a substrate formed from an aluminum material;
forming a zinc material underlayer on a surface of said substrate; and
forming an aluminum coating on said zinc material underlayer,
wherein said substrate is a fan blade used in a turbine engine,
and wherein the zinc material underlayer has a thickness of from about 0.01 µm to less than 10 µm and said aluminum coating has a thickness in the range of from 5 µm to 50 µm.

9. The method of claim 8, wherein said underlayer forming step comprises depositing a zinc or zinc alloy on said surface using at least one zincating process.

10. The method of claim 8 or claim 9, further comprising plating zinc or a zinc alloy onto said deposited zinc or zinc alloy.

11. The method of any of claims 8-10, wherein said aluminum coating forming step comprises depositing aluminum or an aluminum alloy onto said underlayer.

12. The method of any of claims 8-11, wherein said aluminum coating forming step comprises electroplating aluminum onto said underlayer.

13. The method of any of claims 8-12 wherein said coating forming step comprises chromate conversion coating or trivalent chromium process (TCP) treatment of the aluminium coating as a passivation method.

## Patentansprüche

1. Beschichtungssystem für ein Aluminiumbauteil, das Folgendes umfasst:
ein Substrat, das aus einem Aluminiummaterial gebildet ist;
eine Zinkmaterialopferschicht, die sich auf dem Substrat ablagert; und
eine Aluminiumbeschichtung, die sich über der Zinkopferschicht ablagert,
wobei das Substrat eine Gebläseschaufel ist, die in einem Turbinentriebwerk verwendet wird, und
wobei die Opferschicht eine Dicke von weniger als 10 µm aufweist und die Aluminiumbeschichtung eine Dicke in dem Bereich zwischen 5 µm und 50 µm aufweist.

2. Beschichtungssystem nach Anspruch 1, wobei die Opferschicht Zink ist.

3. Beschichtungssystem nach Anspruch 1, wobei die Opferschicht eine Zinklegierung ist.

4. Beschichtungssystem nach einem der vorstehenden Ansprüche, wobei das Substrat eine Aluminiumlegierung ist.

5. Beschichtungssystem nach einem der vorstehenden Ansprüche, wobei die Aluminiumbeschichtung reines Aluminium ist.

6. Beschichtungssystem nach einem der vorstehenden Ansprüche, wobei die Aluminiumbeschichtung eine elektroplattierte Aluminiumbeschichtung ist.

7. Beschichtungssystem nach einem der vorstehenden Ansprüche, wobei das Substrat ein Turbinentriebwerksbauteil ist.

8. Verfahren zum Bilden eines Beschichtungssystems, das die Korrosionsresistenz verbessert, wobei das Verfahren die folgenden Schritte umfasst:
Bereitstellen eines Substrats, das aus einem Aluminiummaterial gebildet ist;
Bilden einer Zinkmaterialunterschicht auf einer Oberfläche des Substrats; und
Bilden einer Aluminiumbeschichtung auf der Zinkmaterialunterschicht,
wobei das Substrat eine Gebläseschaufel ist, die in einem Turbinentriebwerk verwendet wird,
und wobei die Zinkmaterialunterschicht eine Dicke zwischen etwa 0,01 µm und weniger als 10 µm aufweist und die Aluminiumbeschichtung eine Dicke in dem Bereich zwischen 5 µm und 50 µm aufweist.

9. Verfahren nach Anspruch 8, wobei der Schritt des Bildens der Unterschicht das Ablagern von Zink oder einer Zinklegierung auf der Oberfläche mithilfe mindestens eines Zinkatprozesses umfasst.

10. Verfahren nach Anspruch 8 oder 9, ferner umfassend ein Plattieren von Zink oder einer Zinklegierung auf dem abgelagerten Zink oder der Zinklegierung.

11. Verfahren nach einem der Ansprüche 8-10, wobei der Schritt des Bildens einer Aluminiumbeschichtung ein Ablagern von Aluminium oder einer Aluminiumlegierung auf die Unterschicht umfasst.

12. Verfahren nach einem der Ansprüche 8-11, wobei der Schritt des Bildens einer Aluminiumbeschichtung ein Elektroplattieren von Aluminium auf die Unterschicht umfasst.

13. Verfahren nach einem der Ansprüche 8-12, wobei der Schritt des Bildens einer Beschichtung eine Chromatierung oder eine trivalente Chromprozessbehandlung (trivalent chromium process treatment - TCP-Behandlung) der Aluminiumbeschichtung als ein Passivierungsverfahren umfasst.

## Revendications

1. Système de revêtement pour un composant d'aluminium qui comprend :
un substrat formé à partir d'un matériau en aluminium ;
une couche sacrificielle de matériau de zinc déposée sur ledit substrat ; et
un revêtement d'aluminium déposé sur ladite couche sacrificielle de zinc,
dans lequel ledit substrat est une pale de ventilateur utilisée dans un moteur à turbine, et
dans lequel ladite couche sacrificielle a une épaisseur inférieure à 10 µm et ledit revêtement d'aluminium a une épaisseur comprise dans la plage allant de 5 µm à 50 µm.

2. Système de revêtement selon la revendication 1, dans lequel ladite couche sacrificielle est du zinc.

3. Système de revêtement selon la revendication 1, dans lequel ladite couche sacrificielle est un alliage de zinc.

4. Système de revêtement selon une quelconque revendication précédente, dans lequel ledit substrat est un alliage d'aluminium.

5. Système de revêtement selon une quelconque revendication précédente, dans lequel ledit revêtement d'aluminium est de l'aluminium pur.

6. Système de revêtement selon une quelconque revendication précédente, dans lequel ledit revêtement d'aluminium est un revêtement d'aluminium galvanisé.

7. Système de revêtement selon une quelconque revendication précédente, dans lequel ledit substrat est un composant de moteur à turbine.

8. Procédé de formation d'un système de revêtement qui améliore la résistance à la corrosion comprenant les étapes :
de fourniture d'un substrat formé à partir d'un matériau en aluminium ;
de formation d'une sous-couche de matériau de zinc sur une surface dudit substrat ; et
de formation d'un revêtement d'aluminium sur ladite sous-couche de matériau de zinc,
dans lequel ledit substrat est une pale de ventilateur utilisée dans un moteur à turbine,
et dans lequel la sous-couche de matériau de zinc a une épaisseur comprise entre environ 0,01 µm et moins de 10 µm et ledit revêtement d'aluminium a une épaisseur comprise dans la plage allant de 5 µm à 50 µm.

9. Procédé selon la revendication 8, dans lequel ladite étape de formation de sous-couche comprend le dépôt de zinc ou d'un alliage de zinc sur ladite surface en utilisant au moins un processus de zingage.

10. Procédé selon la revendication 8 ou la revendication 9, comprenant en outre le placage de zinc ou d'un alliage de zinc sur ledit zinc ou alliage de zinc déposé.

11. Procédé selon l'une quelconque des revendications 8 à 10, dans lequel ladite étape de formation de revêtement d'aluminium comprend le dépôt d'aluminium ou d'un alliage d'aluminium sur ladite sous-couche.

12. Procédé selon l'une quelconque des revendications 8 à 11, dans lequel ladite étape de formation de revêtement d'aluminium comprend la galvanoplastie d'aluminium sur ladite sous-couche.

13. Procédé selon l'une quelconque des revendications 8 à 12, dans lequel ladite étape de formation de revêtement comprend un traitement de revêtement de conversion de chromate ou de processus de chrome trivalent (TCP) du revêtement d'aluminium en tant que procédé de passivation.
